



## 3

ordinary process of serving food and storing the food in a refrigerator.

The electroplating according to the invention is carried out in a cyanide water bath which of course is maintained alkaline, for example, in the presence of sodium or potassium hydroxide, that is in the concentration of 7 to 20 grams per liter. The pH of the plated bath is preferably maintained at about 11.5 to 12.5.

The electrolyte has dissolved in it soluble salts providing tin ion, silver ion and nickel ion. In order to create such ions in the bath, the respective cyanides may be introduced or any well-known techniques may be used. For example stannous chloride may be placed in the bath and dissolved by adding sodium cyanide. It will, of course, be evident that the conductivity of the bath can be increased if desired by adding sodium cyanide or other alkali conducting salts.

It is very desirable to maintain a proper balance of the concentration of tin ion, the concentration of silver ion and the concentration of nickel ion as suggested below.

The bath temperature can vary widely, but good results are obtained by plating in a temperature range between 125° F. and 155° F.

The voltage employed will suitably be in the range of 2 to 12 volts direct or unidirectional current. The current density will typically vary between 5 and 60 amperes per square foot, and preferably between 25 and 60 amperes per square foot. For best results a combination of insoluble and soluble anodes may be used, such as soluble anodes of silver and tin and an insoluble anode of stainless steel, platinum, titanium or carbon (graphite). The ratio of areas of anode to cathode should not exceed 1 to 1.

The alloy obtained is an alloy of tin, silver and nickel. It may have the following weight proportions:

| Component                                  | Broad   | Narrow  | Preferred |
|--------------------------------------------|---------|---------|-----------|
| Tin.....                                   | 20-45   | 25-45   | 25-30     |
| Silver.....                                | 45-70   | 50-70   | 65-70     |
| Nickel and a small amount of impurity..... | Balance | Balance | Balance   |

The percent of impurities in these alloys is not in excess of 0.50% (by weight).

## Example 1

The following electrolyte bath was made up in water:

|                        | Grams per liter |
|------------------------|-----------------|
| Tin ion .....          | 5.3             |
| Silver ion .....       | 0.65            |
| Nickel ion .....       | 0.13            |
| Sodium hydroxide ..... | 15              |
| Sodium cyanide .....   | 100             |

Tin was added as tin hydroxide. The silver was added as silver cyanide. The nickel was added as nickel hydroxide.

Components suitable for jewelry and the like were made up consisting of low carbon steel, copper and brass. The components were cleaned of grease, foreign matter and oxide as well known in the procedure described in 2 Metals Handbook (8th Ed. 1964) 307 and following.

The bath was heated to 130° F. plus or minus 5° F., and maintained within that temperature range with constant stirring. An insoluble anode of stainless steel and a soluble anode of silver were used, with an anode to cathode ratio of 1 to 1. The work was inserted as cathode and direct current was supplied between the anode and the cathode under a direct voltage of 1 to 1.5 volts at a current density of 15.0 amperes per square foot. The work

## 4

was electropated for 60 seconds in the above bath under the above conditions, and a deposit was obtained which was silvery white and bright without burnishing. No porosity was visible, and the coating was tarnish-free after immersion in a 10% water solution of sodium sulfide for 5 minutes.

Spectrographic analysis showed that the electrodeposit had the following composition by weight:

|                             |               |    |
|-----------------------------|---------------|----|
| Tin .....                   | percent ..... | 26 |
| Silver .....                | do .....      | 70 |
| Nickel and impurities ..... | Balance       |    |

## Example 2

In order to make an alloy of higher tin content the preferred technique is to increase the bath temperature and plate at higher current density.

The procedure of Example 1 was followed except that the bath temperature was maintained at 140° F. plus or minus 5°, and the work was plated at a current density of 45 amperes per square foot. The alloy deposit in this case had the following composition by weight:

|                             |               |    |
|-----------------------------|---------------|----|
| Tin .....                   | percent ..... | 45 |
| Silver .....                | do .....      | 45 |
| Nickel and impurities ..... | Balance       |    |

For a discussion of control of alloy content by temperature and current density see 1 Brenner Electrodeposition of Alloys (1963), p. 610, paragraph 19.2b.

## Example 3

By adjusting the temperature and current density I have obtained alloys having intermediate tin contents. Using a bath temperature of 150° F. and a current density of 30 amperes per square foot I have obtained from this bath an alloy of the following composition by weight:

|                             |               |    |
|-----------------------------|---------------|----|
| Tin .....                   | percent ..... | 29 |
| Silver .....                | do .....      | 30 |
| Nickel and impurities ..... | Balance       |    |

## Example 4

By plating at a bath temperature of 120° F. and a current density of 20 amperes per square foot, I have obtained a coating having the following composition by weight:

|                             |               |    |
|-----------------------------|---------------|----|
| Tin .....                   | percent ..... | 30 |
| Silver .....                | do .....      | 69 |
| Nickel and impurities ..... | Balance       |    |

In view of my invention and disclosure, variations and modifications to meet individual whim or particular need will doubtless become evident to others skilled in the art, to obtain all or part of the benefits of my invention without copying the composition and process shown, and I therefore claim all such insofar as they fall within the reasonable spirit and scope of my claims.

Having thus described my invention, what I claim as new and desire to secure by Letters Patent is:

1. An electrolyte for electroplating a bright silver alloy essentially consisting of an alkaline cyanide water bath comprising 3.0 to 30.0 grams per liter of tin ion, 0.3 to 3.0 grams per liter of silver ion, and 0.13 to 1.35 grams per liter of nickel ion.

2. An electrolyte of claim 1, essentially consisting of 5.3 grams per liter of tin ion, 0.65 gram per liter of silver ion and 0.13 gram per liter of nickel ion.

3. A process of electrodepositing a tarnish-inhibited bright silver alloy which comprises establishing an alkaline cyanide water bath in which the concentration of tin ion is between 3.0 and 30.0 grams per liter, the concentration of silver ion is between 0.3 and 3.0 grams per liter and the concentration of nickel ion is between 0.13 and 1.35

grams per liter, without other substantial metal components, and passing a current unidirectionally through the bath between an electrode and the work as cathode to deposit an alloy of tin, silver and nickel, without substantial quantities of other metallic components.

4. The process of claim 3, in which the temperature of the bath is between 120 and 155° F.

5. The process of claim 4, in which the current density is between 5 and 60 amperes per square foot.

6. The process of claim 5, in which the concentration of tin ion is 5.3 grams per liter, the concentration of silver ion is 0.65 gram per liter and the concentration of nickel ion is 0.13 gram per liter.

## References Cited

## UNITED STATES PATENTS

|           |        |          |            |
|-----------|--------|----------|------------|
| 1,404,156 | 1/1922 | Marino   | 204—43     |
| 3,591,370 | 7/1971 | Denereaz | 75—173 R X |

## OTHER REFERENCES

Frederick A. Lowenheim, "Modern Electroplating," pp. 453—455 (1968).

10 GERALD L. KAPLAN, Primary Examiner

U.S. Cl. X.R.

75—173 R